

## UNITED STATES PATENT OFFICE

2,221,250

## MAGNESIUM BASE ALLOY

Joseph D. Hanawalt and John C. McDonald, Midland, Mich., assignors to The Dow Chemical Company, Midland, Mich., a corporation of Michigan

No Drawing. Application November 13, 1939.  
Serial No. 304,127

## 3 Claims. (Cl. 75—168)

The invention relates to magnesium base alloys. It more particularly concerns alloys of this nature having a high degree of formability coupled with other improved physical properties, such as 5 high yield and tensile strengths.

Magnesium base alloys are being widely used in various structural and mechanical arts where a light weight metal is highly desirable, such as for use in making large castings, forgings, and the like. However, the use of these alloys in rolled 10 form to make sheet metal articles requiring forming operations, such as bending, drawing, or the like, has not progressed as rapidly due to the fact that in general alloys of good formability, permitting 15 relatively sharp bends to be made without

have found that in general the preferred combination of properties, such as the most desirable ductility for forming operations associated with high tensile and yield strengths is found in alloys containing from 3 to 5 per cent of thallium and from 0.1 to 0.3 per cent of calcium. 5

The following table, which lists some of the properties of sheet metal made from our new alloy and compares these properties with those of the related binary alloys, illustrates the improvement in yield strength, tensile strength, and ductility or formability, as represented by per cent increase in elongation, of the new alloy over the corresponding properties of the closely related 10 alloys. 15

Table

| 20 | Nominal composition in percent<br>(magnesium—remainder) |      | Annealed                       |                                  |                                | Cold rolled                    |                                  |                                | 20 |
|----|---------------------------------------------------------|------|--------------------------------|----------------------------------|--------------------------------|--------------------------------|----------------------------------|--------------------------------|----|
|    | Ca                                                      | Tl   | Yield strength in lbs./sq. in. | Tensile strength in lbs./sq. in. | Percent elongation in 2 inches | Yield strength in lbs./sq. in. | Tensile strength in lbs./sq. in. | Percent elongation in 2 inches |    |
| 25 | 0.3                                                     | 0.3  | 17,000                         | 30,000                           | 13                             | 27,000                         | 32,000                           | 2                              | 25 |
|    | 0.2                                                     | 0.3  | 18,000                         | 32,000                           | 3                              | 22,000                         | 29,000                           | 2                              |    |
|    | 0.2                                                     | 1.0  | 17,000                         | 32,000                           | 14                             | 27,000                         | 32,000                           | 7                              |    |
|    | 0.3                                                     | 1.0  | 19,000                         | 32,000                           | 3                              | 26,000                         | 31,000                           | 2                              |    |
|    | 0.3                                                     | 3.0  | 18,000                         | 32,000                           | 15                             | 28,000                         | 34,000                           | 2                              |    |
|    | 0.2                                                     | 3.0  | 20,000                         | 32,000                           | 9                              | 24,000                         | 32,000                           | 5                              |    |
|    | 0.2                                                     | 6.0  | 21,000                         | 35,000                           | 14                             | 29,000                         | 37,000                           | 7                              |    |
|    | 0.2                                                     | 6.0  | 20,000                         | 34,000                           | 11                             | 31,000                         | 34,000                           | 2                              |    |
| 30 | 0.2                                                     | 10.0 | 20,000                         | 32,000                           | 15                             | 31,000                         | 36,000                           | 4                              | 30 |
|    | 0.2                                                     | 10.0 | 19,000                         | 34,000                           | 15                             | 26,000                         | 32,000                           | 6                              |    |

35 the articles developing external cracks, usually have inferior characteristics as regards their tensile and yield strengths.

It is accordingly the principal object of the invention to provide a magnesium base alloy which 40 may be made into rolled sheet or the like, possessing a sufficient degree of formability or ductility to be sharply bent, drawn, or otherwise shaped, while having high tensile and yield strengths.

45 Other objects and advantages will be apparent as the description of the invention proceeds.

Our invention resides in the discovery that a magnesium base alloy composed of from 0.1 to 10 per cent of thallium and from 0.05 to 1 per cent 50 of calcium, the balance being substantially all magnesium, is endowed with the afore-mentioned properties. While the properties of improved formability or ductility associated with high tensile and yield strengths are manifest over the entire range of composition above indicated, we

35 The properties listed in the above table under the section headed by the term "annealed" were obtained by first rolling the alloys at a temperature between about 600° to 700° F., and thereafter annealing them at various temperatures through a temperature range of from 400° to 800° 40 F. The properties selected for the table were those of the annealed specimens which exhibited the maximum elongation. The properties listed under the section headed "cold rolled" were obtained by subjecting specimens of the alloys which had been hot rolled at a temperature of from 600° to 700° F. to additional rolling in the cold state, to bring about a total reduction in thickness of from 2 to 10 per cent. The properties selected for the table were those of the cold rolled specimens which showed the greatest tensile and yield strengths, while having at least a 1 per cent elongation in 2 inches. 45

By comparison of the properties set forth in 55

the above table it will be observed that in almost every instance every property of the new ternary alloy is superior to those of the parent binary alloys having similar percentages of the alloying ingredient present. Further, it will be observed that the combined properties of the new alloy are always superior to those of the parent alloys.

5 While the new alloy is most useful in wrought form, such as sheets, due to its formability characteristics it may also be suitably used in making 10 castings, forgings, extruded forms, and the like.

15 The new alloy may be compounded in any of the ways known to the art, such as by adding the alloying constituents to the molten magnesium under a suitable flux. The flux should be substantially free of magnesium chloride if the calcium content is to be above 0.3 per cent. In those instances where an alloy is to be compounded containing less than 0.3 per cent of calcium, mag-

nesium chloride may be present in the flux without exerting a deleterious effect. In the latter case, however, it is usually preferable to add the calcium last without too much stirring or agitation in order that the loss of calcium into the 5 flux will be substantially prevented.

We claim:

1. A magnesium base alloy containing from 0.1 to 10 per cent of thallium and from 0.05 to 1.0 per cent of calcium, the balance being mag- 10 nesium.

2. A magnesium base alloy containing from 3 to 5 per cent of thallium and from 0.1 to 0.3 per cent of calcium, the balance being magnesium.

3. A magnesium base alloy consisting of ap- 15 proximately 4 per cent of thallium and 0.2 per cent of calcium, the balance being magnesium.

JOHN C. McDONALD.

JOSEPH D. HANAWALT.